

# United States Patent Office

2,920,954  
Patented Jan. 12, 1960

1

2,920,954

## STAINLESS STEEL ALLOY OF HIGH HARDNESS

Norman S. Mott, Westfield, N.J., assignor to Cooper Alloy Corporation, Hillside, N.J., a corporation of New Jersey

No Drawing. Application April 15, 1958  
Serial No. 728,556

9 Claims. (Cl. 75—128)

This invention relates to stainless steel alloys, and 15 more particularly to such an alloy which is characterized by very high hardness.

The primary object of the present invention is to generally improve precipitation hardenable stainless steel alloys, especially alloys of the chromium-nickel-molybdenum type. A more particular object is to provide such an alloy which may be hardened to a very high degree of hardness. By that I mean a Brinell number no lower than 400, and preferably 500 or more. A further object is to provide such an alloy which is accompanied by the 25 excellent corrosion-resistance of the well-known AISI 316 and 317 types of stainless steel.

The new alloy is based on the simultaneous use of columbium and an increased amount of silicon. If desired, the nitrogen content also may be increased, as hereinafter explained, but this is optional and is unimportant compared to the use of columbium and increased silicon.

The broad range of my alloy includes the following chemical composition:

|                | Percent                |
|----------------|------------------------|
| C              | 1.08                   |
| Cr             | 18-30                  |
| Ni             | 8-12                   |
| Mo             | 2-6                    |
| Si             | 3-6                    |
| Cb             | 0.50-1.50              |
| N <sub>2</sub> | <sup>2</sup> 0.04-0.25 |

<sup>1</sup> Maximum.

<sup>2</sup> Optional.

In respect to nitrogen a normal minimum residual is considered to be 0.04%. Therefore, at the minimum there is no intentional addition of nitrogen.

A closer and more preferred range is as follows:

|                | Percent                |
|----------------|------------------------|
| C              | 1.08                   |
| Cr             | 18-21                  |
| Ni             | 8-12                   |
| Mo             | 3.75-4.25              |
| Si             | 3.5-5.0                |
| Cb             | 0.75-1.25              |
| N <sub>2</sub> | <sup>2</sup> 0.04-0.15 |

<sup>1</sup> Maximum.

<sup>2</sup> Optional.

In both of the chemical composition ranges given above, the balance would be iron, manganese, sulfur, phosphorus and other elements incidental to manufacture and normally found as residuals in stainless steel alloys.

Four specific examples of my alloy are given in the following table:

2  
Table I

|    | Test No.          | X-18DC | X-18DE | X-18D | X-18DF |
|----|-------------------|--------|--------|-------|--------|
| 5  | C percent         | .056   | .053   | .058  | .049   |
|    | Cr do             | 20.08  | 20.21  | 20.35 | 20.01  |
|    | Ni do             | 8.56   | 8.81   | 8.60  | 8.69   |
|    | Mn do             | .88    | .79    | .88   | .85    |
|    | Mo do             | 3.92   | 3.78   | 3.78  | 3.82   |
|    | Si do             | 4.89   | 3.49   | 4.97  | 3.56   |
|    | Cb do             | .54    | .06    | .86   | 1.23   |
| 10 | N <sub>2</sub> do | 1.043  | .12    | 1.041 | 1.041  |
|    | BHN WQ            | 351    | 332    | 387   | 418    |
|    | BHN PH            | 512    | 512    | 555   | 600    |

<sup>1</sup> Not intentionally added.

In the above and in all following tables "BHN" means Brinell hardness number; "WQ" means water quenched from 2000° F.; and "PH" means precipitation hardened by holding at 850°-925° F. for eight hours, and then furnace cooling.

20 It will be noted that the above specific examples of my alloy all have a remarkable hardness of over 500 BHN in the PH condition.

To show the effect of adding columbium, the following table may be referred to. The test number X-18DF is repeated from Table I.

Table II

|    | Test No.          | X-18  | X-18DA | X-18DB | X-18DF |
|----|-------------------|-------|--------|--------|--------|
| 30 | C percent         | .033  | .049   | .052   | .049   |
|    | Cr do             | 20.25 | 20.26  | 20.10  | 20.01  |
|    | Ni do             | 8.90  | 8.34   | 8.60   | 8.69   |
|    | Mn do             | .86   | .81    | .89    | .85    |
|    | Mo do             | 3.96  | 3.89   | 3.96   | 3.82   |
|    | Si do             | 3.46  | 3.51   | 3.55   | 3.56   |
|    | Cb do             | .00   | .51    | .98    | 1.23   |
| 35 | N <sub>2</sub> do | .037  | .039   | .040   | .041   |
|    | BHN WQ            | 262   | 286    | 302    | 418    |
|    | BHN PH            | 341   | 418    | 495    | 600    |

The elements other than columbium are substantially constant. This table shows that increasing the columbium percentage increases the hardness at a substantially constant level of the other elements. I consider a BHN of 400 in the PH condition the lowest hardness desirable for the present objective, and I consider a BHN of 500 preferable. A BHN of 600 is an upper limit of hardness, because above that cracks are produced. Accordingly, a range of 0.50 to 1.50% columbium is indicated, while a more preferred or narrower range would be 0.75 to 1.25% for the columbium. It may be noted that in these tests the silicon was approximately 3.50%. Incidentally, test X-18DB could have been included in Table I as showing a fifth example of my invention.

45 The effect of increasing the nitrogen content is shown in the following table:

Table III

|    | Test No.          | X-18DB | X-18DE |
|----|-------------------|--------|--------|
| 60 | C percent         | .052   | .053   |
|    | Cr do             | 20.10  | 20.21  |
|    | Ni do             | 8.60   | 8.81   |
|    | Mn do             | .89    | .79    |
|    | Mo do             | 3.96   | 3.76   |
|    | Si do             | 3.55   | 3.49   |
|    | Cb do             | .98    | .96    |
|    | N <sub>2</sub> do | .040   | .120   |
|    | BHN WQ            | 302    | 332    |
|    | BHN PH            | 495    | 512    |

The elements other than nitrogen are substantially constant. This table shows that increasing the nitrogen content will assist in increasing the BHN hardness, but to only a minor degree as compared with increasing columbium and silicon. Therefore, an increase of nitrogen over the usual amount found in normal melting practice, say, 0.06%, is optional. I recommend 0.25% as the upper level, because above that there is difficulty with metal gassing.

The effect of increasing silicon is shown in the following table:

Table IV

| Test No.                    | X-18DA | X-18DC | X-18DB | X-18D |
|-----------------------------|--------|--------|--------|-------|
| C.....percent.....          | .049   | .056   | .052   | .058  |
| Cr.....do.....              | 20.26  | 20.08  | 20.10  | 20.35 |
| Ni.....do.....              | 8.34   | 8.56   | 8.60   | 8.60  |
| Mn.....do.....              | .81    | .88    | .89    | .83   |
| Mo.....do.....              | 3.89   | 3.92   | 3.96   | 3.78  |
| Si.....do.....              | 3.51   | 4.89   | 3.55   | 4.97  |
| Cb.....do.....              | .51    | .54    | .98    | .86   |
| N <sub>2</sub> .....do..... | .039   | .043   | .040   | .041  |
| BHN WQ.....                 | 286    | 351    | 302    | 387   |
| BHN PH.....                 | 418    | 512    | 495    | 555   |

The first two tests are with a low level of columbium, while the second two are with a high level of columbium. Otherwise, the elements are unchanged, except for silicon, which is changed from about 3.5 to 5.0%.

This table shows the effect of increasing silicon on the BHN hardness values. Since a BHN of 400 minimum is my objective, it will be seen that a silicon content of about 3.5% is necessary at the lower columbium level of about 0.5%. A silicon content of about 3% is necessary at the higher columbium level of about 1.0%. Above 5% silicon, embrittlement and a tendency towards cracking sets in, and I have therefore set a maximum of 6%, with a preferred limit of 5%, for this element.

In all of the foregoing analyses, the iron content is not included, but it is understood that the balance is iron, subject to the presence of small amounts of impurities incidental to the usual melting practice when dealing with ferrous metals. The maximum carbon content should be no higher than say 0.08%.

It will be understood that the alloys are fully resistant to the usual corrosion tests, specifically 65% boiling nitric acid, 50% sulphuric acid at 80° F., and 5% hydrochloric acid at 80° F. These alloys are also fully resistant to salt spray. As previously indicated, in this respect the present alloys, despite their very high hardness, are comparable to the well-known AISI 316 and 317 types of stainless steel.

The alloys are weldable by using welding rods of the same general composition as the alloy being welded. These alloys are soft enough in the quench-annealed condition to be readily machinable, and they may be precipitation hardened by a comparatively low-temperature heat-treatment to a very high degree of hardness.

It will be apparent that while I have set forth specific examples of my improved alloys, changes may be made without departing from the scope of the invention as sought to be defined in the following claims.

I claim:

1. A precipitation hardenable stainless steel alloy of very high hardness having a hardness exceeding 400 BHN in the precipitation hardened state, said alloy having a range of 18% to 30% chromium, 8% to 12% nickel, 2% to 6% molybdenum, 3% to 6% silicon, 0.5% to 1.5% columbium, and a carbon content not exceeding 0.08%, the remainder being essentially iron.

2. A precipitation hardenable stainless steel alloy of very high hardness having a hardness exceeding 400 BHN in the precipitation hardened state, said alloy having a range of 18% to 30% chromium, 8% to 12% nickel, 2% to 6% molybdenum, 3% to 6% silicon, 0.5% to

1.5% columbium, and a carbon content not exceeding 0.08%, the remainder being essentially iron, with manganese, sulphur, phosphorus, and other elements incidental to manufacture and normally found as residuals in stainless steel alloys, and an optional nitrogen content of 0.04% to 0.25%.

3. A precipitation hardenable stainless steel alloy of very high hardness having a hardness exceeding 400 BHN in the precipitation hardened state, said alloy having a range of 18% to 21% chromium, 8% to 12% nickel, 3.75% to 4.25% molybdenum, 3.5% to 5.0% silicon, 0.75% to 1.25% columbium, and a carbon content not exceeding 0.08%, the remainder being essentially iron,

4. A precipitation hardenable stainless steel alloy of very high hardness having a hardness exceeding 400 BHN in the precipitation hardened state, said alloy having a range of 18% to 21% chromium, 8% to 12% nickel, 3.75% to 4.25% molybdenum, 3.5% to 5.0% silicon, 0.75% to 1.25% columbium, and a carbon content not exceeding 0.08%, the remainder being essentially iron, with manganese, sulphur, phosphorus, and other elements incidental to manufacture and normally found as residuals in stainless steel alloys, and an optional nitrogen content of 0.04% to 0.15%.

5. A precipitation hardenable stainless steel alloy of very high hardness having a hardness exceeding 400 BHN in the precipitation hardened state, said alloy having approximately 20.08% chromium, 8.56% nickel, 0.88% manganese, 3.92% molybdenum, 4.89% silicon, 0.54% columbium, 0.043% nitrogen, and 0.056% carbon, the remainder being essentially iron and other elements incidental to manufacture and normally found as residuals in stainless steel alloys.

6. A precipitation hardenable stainless steel alloy of very high hardness having a hardness exceeding 400 BHN in the precipitation hardened state, said alloy having approximately 20.21% chromium, 8.81% nickel, 0.79% manganese, 3.76% molybdenum, 3.49% silicon, 0.96% columbium, 0.12% nitrogen, and 0.053% carbon, the remainder being essentially iron and other elements incidental to manufacture and normally found as residuals in stainless steel alloys.

7. A precipitation hardenable stainless steel alloy of very high hardness having a hardness exceeding 400 BHN in the precipitation hardened state, said alloy having approximately 20.35% chromium, 8.6% nickel, 0.83% manganese, 3.78% molybdenum, 4.97% silicon, 0.86% columbium, 0.041% nitrogen, and 0.058% carbon, the remainder being essentially iron and other elements incidental to manufacture and normally found as residuals in stainless steel alloys.

8. A precipitation hardenable stainless steel alloy of very high hardness having a hardness exceeding 400 BHN in the precipitation hardened state, said alloy having approximately 20.01% chromium, 8.69% nickel, 0.85% manganese, 3.82% molybdenum, 3.56% silicon, 1.23% columbium, 0.041% nitrogen, and 0.049% carbon, the remainder being essentially iron and other elements incidental to manufacture and normally found as residuals in stainless steel alloys.

9. A precipitation hardenable stainless steel alloy having a hardness exceeding 400 BHN in the precipitation hardened state, said alloy having approximately 20.10% chromium, 8.60% nickel, 0.89% manganese, 3.96% molybdenum, 3.55% silicon, 0.98% columbium, 0.04% nitrogen, and 0.052% carbon, the remainder being essentially iron and other elements incidental to manufacture and normally found as residuals in stainless steel alloys.

70 References Cited in the file of this patent

UNITED STATES PATENTS

2,403,128 Scott et al. \_\_\_\_\_ July 2, 1946  
2,822,265 Eberle et al. \_\_\_\_\_ Feb. 4, 1958